

# UNITED STATES PATENT OFFICE.

PAUL DHÉ, OF PARIS, FRANCE.

FILAMENT COMPOSED OF BASALT.

No Drawing.

Application filed April 15, 1921. Serial No. 461,641.

*To all whom it may concern:*

Be it known that I, PAUL DHÉ, a citizen of the Republic of France, and residing at Paris, Seine Department, No. 124 Rue 5 de Provence, in the Republic of France, engineer, have invented certain new and useful Filaments Composed of Basalt, of which the following is a specification.

This invention relates to a method for 10 the use of basalt wherein the basalt is melted and is transformed when in a pasty condition into fine threads. These latter have very flexible character and may be substituted for textile fibres for a great number 15 of uses. The threads may be employed alone, or in combination with other threads or fibres, in the manufacture of fabrics, cables, cords, trolley supports, submarine cables, and the like. Basalt threads thus 20 prepared are advantageous in that they are not attacked by the major part of chemical substances and are excellent non-conductors of electricity.

The threads are easily obtained by drawing out melted basalt, for instance after 25

the same manner as threads of glass or like material are produced. It is advantageous to maintain the thread for a certain time at a temperature in proximity to 800° C. and to avoid all sudden cooling, and in this 30 manner a wire having a de-vitrified texture and a great flexibility may be obtained.

## Claims.

1. As a new product, a filament for the manufacture of fabrics, cables, cords and 35 other textile articles, said filament being constituted by basalt which is melted and subjected to the drawing process.

2. As a new product, a filament for the manufacture of fabrics, cables, cords and 40 other textile articles, said filament being constituted by basalt which is melted and subjected to the drawing process and is given a crystalline structure by annealing.

In testimony that I claim the foregoing 45 as my invention I have signed my name in presence of the subscribing witness.

PAUL DHÉ.

Witness:

MAURICE ROUX.